

March 23, 1954

R. K. STRATFORD ET AL  
SYNTHETIC LUBRICATING OIL

2,673,175

Filed April 21, 1951



MEANING OF SYMBOLS

MCL 10 = MID-CONTINENT LOUDON  
S.A.E. 10 GRADE

MCL 30 = MID-CONTINENT LOUDON  
S.A.E. 30 GRADE

CWO = COLUMBIAN WEBSTER  
LIGHTER THAN S.A.E. 10 GRADE

CW 30 = COLUMBIAN WEBSTER  
SAE 30 GRADE

50/100 PFFE. DIST. (MCL) = PARAFFIN DISTILLATE  
OF 50 SUS VISCOSITY AT 100° F. FROM  
MID-CONTINENT LOUDON CRUDE.

Reginald K. Stratford  
Frank A. Stuart  
William A. Jones Inventors

By g.t. small attorney

## UNITED STATES PATENT OFFICE

2,673,175

## SYNTHETIC LUBRICATING OIL

Reginald K. Stratford, Corunna, Ontario, and  
 William A. Jones, Sarnia, Ontario, Canada, and  
 Frank A. Stuart, Richmond, Calif., assignors  
 to Standard Oil Development Company, a cor-  
 poration of Delaware

Application April 21, 1951, Serial No. 222,172

14 Claims. (Cl. 196—142)

1

This invention relates to the manufacture of a synthetic lubricating oil of improved properties by chemical treatment of a refined mineral lubricating oil fraction.

The invention will be described hereinafter with reference to the accompanying drawing, the single figure of which is a graphical illustration of the relative utility of various oils for the purposes of the present invention.

In the operation of internal combustion engines, particularly at relatively low crankcase and cooling jacket temperatures, deposition of varnish on piston surfaces, oil screen and other engine parts is a serious problem. This varnish deposition which is mainly caused by the fuel and varies with the type of fuel used as well as with engine operating conditions, may be controlled by lubricants which have high solubility for oxidized fuel combustion products and/or prevent deposition of insoluble polymerization products. It is a well-known practice to add oxidation inhibitors to oil in order to prevent lubricating oil oxidation in high temperature operation. Such inhibitors, however, generally do not lessen varnish formation from fuel products in low temperature operation and, in fact, sometimes increase the amount of varnish formation. In order to keep sludge and insoluble matter in suspension it is a common practice to use agents known as detergents in combination with inhibitors. In general, detergent additives do not increase the solvent power of the lubricant for varnish forming materials. Hence the concentrations generally used do not give effective reduction of varnish deposits.

By the present invention, the mineral lubricating oil is submitted to chemical treatment before addition of antioxidant, if the latter is required. The resulting product not only keeps suspended material in suspension but also inhibits formation of insoluble varnish. At the same time the chemical treatment gives a product of higher viscosity than the original mineral oil. Thus, by the treatment it is possible to increase the viscosity to that desired for lubricating purposes, without the necessity of adding thickeners or without employing more expensive base stocks, such as bright stocks. Products obtained by the process of the present invention have shown marked ability to prevent deposition of varnish when employed in the crankcase of a typical automobile engine, operating under conditions at which varnish formation is heavy when mineral lubricants and a deposit forming fuel are used.

Briefly, the process of the present invention

involves the treatment of a phenol extracted, hydrofinished mineral lubricating oil with oxygen to produce a material having a saponification number of at least 20, substantially reducing the neutralization number of the resulting product by means of a neutralizing agent, and preferably though not always necessarily adding to the neutralized product an antioxidant to prevent further oxidation. Whether or not an antioxidant is necessary is dependent on the nature of the base stock processed and the manner of oxidation.

The method of the invention may be applied generally to distillates in the viscosity range from heavy gas oil (30 seconds viscosity Saybolt at 100° F.) to heavy lubricating oil distillates (3000 seconds Saybolt at 100° F.). For example, distillates from Mid-Continent (Louden) and Colombian crudes have been found to be quite suitable.

It is considered necessary, prior to oxidation, to apply phenol extraction and mild hydrogenation to the base oil, for the purpose of obtaining a material which oxidizes rapidly without the formation of oil insoluble sludge. Dewaxing may also be applied, but this is not essential. The scope of the process is not limited however to the use of phenol extraction and mild hydrogenation as the method of preparing a base oil suitable for oxidation. It is considered possible by proper choice of conditions to produce a suitable base stock by refining the lubricating oil distillate by means of other extracting solvents such as furfural, cresols, nitrobenzene, etc. and hydrofinishing or by fuming acid treatment or by treatment with silica gel or by severe hydrogenation followed by mild hydrogenation.

The solvent extracted distillate may be hydrogenated, preferably by the use of nickel, nickel on kieselguhr, platinum or palladium catalysts, but it is also possible to use sulfur resistant catalysts, such as nickel-tungsten sulfides, cobalt molybdate or alumina, molybdenum on alumina and other known hydrogenation catalysts. The degree of hydrogenation necessary and the hydrogenation conditions depend on the nature of the distillate being refined and the degree of extraction to which it has been subjected. It is desirable but not absolutely necessary to decrease the sulfur content of the oil to 0.03% or lower and to improve the color to about 18 Robinson or better by the hydrogenation process.

The oxidation step is carried out by passing oxygen or air into the oil, preferably through a diffuser placed in the oil contained in a tall

column reactor to allow intimate contact. The degree of oxidation of the oil may be conveniently measured by the increase in saponification number, which is approximately proportional to the amount of oxygen absorbed. At the same time the viscosity is increased and the aniline point is decreased. Products oxidized to a saponification number of about 20 to as high as about 70 or over and subsequently treated as described below have been found to be effective in decreasing piston varnish formation. The preferred temperature range for oxidation is from about 275° F. to about 350° F., although it is possible to carry out the oxidation satisfactorily in the temperature range from about 200° to about 400° F. The saponification number is increased to approximately 20 after an absorption of 8-10% by weight of oxygen and to approximately 50-60 after the absorption of 14-16% oxygen. Yields of oxidized material on the basis of mineral oil charged are generally about 99 volume percent at 20 saponification number and 96 volume percent at 50 saponification value. The exact chemical nature of the saponifiable material cannot be defined from the data at present available.

In the present process no advantage has been demonstrated for the use of metallic catalysts such as manganese naphthenate, calcium salts and other recommended oxidation catalysts. If metallic catalysts are used, extra processing steps may be necessary for their removal. As a catalyst to initiate oxidation, particularly when air is used as the oxidizing agent, benzoyl peroxide has been found to be effective. Other organic peroxides appear to be useful in a similar manner, and do not require the extra processing steps which are required when metal catalysts are used.

Oxidation by means of air takes place much more slowly of course than with gaseous oxygen. Whereas a hydrofinished Mid-Continent Louden stock was converted by commercial oxygen at 350° F. into a material having a saponification number of 25-30 in 45 minutes, similar treatment of this stock at the same temperature with air required 54 hours to produce a similar result. Oxidation was accomplished by means of air at 400° F. in 16 hours, but the product was very dark in color. The addition of 1% benzoyl peroxide as catalyst in the air treatment at 300° F. produced an oxidized product of 43 saponification number in 4 hours.

Following the oxidation step, which produces an acidic product, a basic material is added to substantially reduce the acidity. Generally the amount of neutralizing agent which is added is that which is theoretically sufficient to reduce the neutralization number to 0. In actual practice a zero neutralization value has not been obtained by using the theoretical quantity of basic material. However, a certain degree of acidity can be tolerated. The addition of the theoretically required amount of neutralizing agent has been found to give a product which is non-corrosive to iron and babbitt at temperatures up to 350° F. It is desirable to reduce the original neutralization number, as determined by ASTM Method D663-46T, of the oxidized product to a value not greater than one-half the original value. In the average case the neutralization number of the product should not be greater than about 6. However, a good product has been obtained by oxidizing sufficiently to raise the neutralization number to about 21 and then treating with a neutralizing agent (butyl alcohol) in at least

and preferably greater than theoretical quantity even though the final neutralization number was 9.4. It appears to be necessary to reduce the neutralization number by at least half, and preferably more than half.

As neutralizing agents alcohols, such as butyl alcohol, as well as metallic bases have been used. The alcohol has the advantage of not introducing metallic constituents into the oil, and even where metal bases are used alcohol is useful for partially reducing high neutralization value in order to avoid the necessity of adding an undesirably large amount of metallic bases. Metallic bases, such as the oxides and hydroxides of alkaline earth metals, are then used as neutralizing agents. These give a product which has the ability to keep solid sludge and water in suspension.

For this purpose, calcium hydroxide in combination with calcium oxide has been used, the purpose of the calcium oxide being to react with the water formed by the action of calcium hydroxide. Similarly, barium hydroxide with and without barium oxide has been used. Magnesium hydroxide and/or oxide is also believed to be suitable. Sodium and aluminum hydroxides were not found to be satisfactory because of a thickening action on the product.

The practice in using volatile alcohols such as butyl is to heat oxidized material with 5 to 10 times as much alcohol as is theoretically required for complete reduction of the neutralization value by esterification. During the heating period part of the alcohol is gradually distilled off in order to remove water and promote esterification. Organic amines and ammonia may be employed in place of alcohols. Any of the aliphatic saturated alcohols of 2 to 20 carbon atoms may be used; those of 3 to 8 carbon atoms are preferred.

The practice in using metallic bases with or without prior neutralization by alcohol is to add the calculated theoretical amount of the base to the oxidized material, and to heat preferably to about 150-250° F. with agitation until all the neutralizing material dissolves. The metallic base may be added gradually or all at once.

After partial or complete reduction of the neutralization value by esterification and/or interaction with calcium hydroxide or other suitable metallic bases, final traces of alcohol and/or low boiling oxidation products including water are removed from the oxidized material by vacuum distillation. In the laboratory vacuum distillation has been carried out at 5-10 mm. pressure and the distillate taken overhead until the still temperature reaches 450-500° F. Lower or higher pressures may be employed provided the corresponding adjustment is made in the final distillation temperature. Exact choice of distillation conditions depends on the viscosity and boiling range of the original distillate. After vacuum distillation the yield of material which is not carried overhead is generally about 94-95 volume percent of a product with 50 saponification number. Yields are 96-97 volume percent of oxidized product when it has a saponification number of about 20. After vacuum stripping, the oxidized and neutralized oil is preferably filtered to remove any suspended material. When pure calcium hydroxide and pure calcium oxide are used as neutralizing agents no suspended material is formed and filtration is not necessary.

It is considered necessary to add to the final product an antioxidant in sufficient amount to reduce the tendency to further oxidation by an

amount which will prevent oxygen absorption at 350° F. at a greater rate than about 1% per hour, as determined by an oxygen absorption test conducted as follows: 10 cc. of oil is placed in a closed tube fitted with an oxygen disperser, immersed in the oil. The tube is placed in a bath maintained at 350° F. and connected to a burette containing oxygen. Oxygen is circulated through the oil at a rate of 750 ml./min. The amount of oxygen in the burette is measured at intervals and the rate of oxygen uptake plotted against time. A satisfactory oil shows only a slow rate of oxygen absorption which does not increase with time.

Any of the well known antioxidants found suitable for use with lubricating oils may be used for this purpose. A particularly satisfactory antioxidant is the reaction product of  $\alpha$ -pinene and phosphorus pentasulfide. Other suitable antioxidants are the alkaline earth metal salts of alkylated phenol sulfides and their reaction products with sulfur and sulfides of phosphorus, also phenyl  $\alpha$ -naphthylamine and 2,6-di-tert.-butyl-4-methylphenol. The last two are recommended for use only where the oil is not subjected to temperatures greater than 300° F.

In the following table are given typical inspections of an oil after the various treatments described above, the original oils being Mid-Continent Louden stocks which have been phenol extracted and hydrofinished.

weight percent of 50% nickel on kieselguhr catalyst. After four hours at 250° F. and two hours at 450° F. a product was obtained in 99% yield having 0.02% sulfur content and +26 Saybolt color. This product was then blown with oxygen at 350° F., whereby 14 weight percent of oxygen was absorbed after 2½ hours. A yield of 97-98 weight percent of oxidized product, based on the oil charge, was obtained of a light red color, having a saponification number of 56 and a neutralization number of 17. The viscosity had increased to 533 seconds Saybolt at 100° F.

This oxidized product was heated with 10 volume percent of butyl alcohol in such a manner as to distill off approximately one-half of the alcohol over a period of 4 hours. The balance of the alcohol was then distilled off by heating the mixture to 450° F. under 10 mm. vacuum. By this treatment the neutralization value was reduced to 10. The residue from the distillation was then heated for six hours with 0.3% calcium hydroxide and 0.15% calcium oxide. After this treatment all the calcium hydroxide and calcium oxide had dissolved in the oil and the neutralization number was reduced to 6. The oil was filtered to remove any suspended undissolved material, but practically no residue was obtained on the filter. The product after neutralization, when blown with oxygen at 350° F., absorbed approximately 1.4 weight percent after one hour. 1.0% of a commercial oxidation inhibitor (reaction

| Oil Designation | Treatment                                                                                              | Vis. (100° F.) | V. I. | Sap. No. | Neut. No. | Aniline Point | Oxygen Absorption (350° F.) |
|-----------------|--------------------------------------------------------------------------------------------------------|----------------|-------|----------|-----------|---------------|-----------------------------|
| A1              | Extracted hydrofinished light lube distillate.                                                         | 150            | 95    | nil      | nil       | 216           | 9% in one-half hour.        |
| A2              | A1 after absorption of 12-14% oxygen.                                                                  | 533            | 64    | 56       | 17        | 156           | 4% in one hour.             |
| A3              | A2 refluxed with butyl alcohol, heated with 0.5% lime at 200° F., 10 hours' vacuum stripped, filtered. | 603            | 80    | 45       | 6         | 154           | 1.4% in one hour.           |
| A4              | A3+1% reaction product $\alpha$ -pinene +P <sub>2</sub> S <sub>5</sub> .                               | 650            | 82    | 45       | 6         | 157           | 0.6% in one hour.           |
| B1              | Extracted hydrofinished light-intermediate lube distillate.                                            | 364            | 95    | nil      | nil       | 228           | 7% in one-half hour.        |
| B2              | B1 after absorption of 8-10% oxygen.                                                                   | 620            | 78    | 23.4     | 7.0       | 195           | 5.5% in one hour.           |
| B3              | B2 heated with 0.4% lime at 200° F., 6 hours' vacuum stripped, filtered.                               | 596            | 89    | 17       | 3.0       | 190           |                             |
| B4              | B3+1% reaction product $\alpha$ -pinene +P <sub>2</sub> S <sub>5</sub> .                               | 602            | 89    | 19.5     | 2.4       | 197           | 0.8% in one hour.           |
| C1              | Medium grade refined distillate.                                                                       | 547            | 64.1  | 68.3     | 21        | 159           |                             |
| C2              | C1 highly oxidized.                                                                                    | 555            | 70    | 70       | 10        | 148           |                             |
| C3              | C2 refluxed with butyl alcohol, heated with 0.5% lime at 200° F., 10 hrs. vacuum stripped, filtered.   | 596            | 70    | 70       | 9.4       | 148           |                             |
| C4              | Same as C3+1% commercial antioxidant.                                                                  |                |       |          |           |               |                             |

In the following examples the preparations of some satisfactory finished products are described in detail, including an engine test of the same, but it is to be understood that these examples are given by way of illustration only and do not limit the scope of the invention.

#### Example 1

A lubricating oil distillate of 165 viscosity (Saybolt) at 100° F., obtained from a Mid-Continent Louden crude was extracted with phenol to a viscosity index (Dean and Davis) of 95, and dewaxed to obtain an A. S. T. M. pour point of 0° F. By this treatment a refined oil was obtained having 0.1% sulfur content and 13 Robinson color. This extracted oil was then blown with oxygen at 350° F., resulting in the absorption of 0.5 weight percent of oxygen in three hours, and the oil had become dark brown in color. The oil was then further treated by hydrogenation at 100 lbs./sq. in. pressure using 10

product of  $\alpha$ -pinene and P<sub>2</sub>S<sub>5</sub>) was then added, and the inhibited oxidized oil when blown with oxygen at 350° F. absorbed only 0.8 weight percent after 3 hours.

The product prepared as described above was tested for 40 hours in a Chevrolet engine operated at 2500 R. P. M. and 45 brake horsepower, at a block temperature of 90° F. and an oil sump temperature of 155° F., using a deposit forming fuel. A similar oil sample, which had undergone the treatments described above, but without the oxidation and neutralization steps, and containing the same amount of oxidation inhibitor, was tested in the same manner. The oils were rated by a demerit system, wherein a perfectly clean surface is given a rating of 0, while a rating of 10 is given to the worst condition which could be expected on that surface, with respect to the deposition of varnish on the piston surfaces. The non-oxidized oil showed a demerit of 5.5-6.5, while the oxidized and

neutralized oil showed a demerit of 0.5 which is quite satisfactory. The oil pan and oil screen of the engine operated on the oxidized lubricant was clean and free of sludge, while the non-oxidized lubricant gave an appreciable quantity 5 of watery sludge and the oil screen was heavily coated with varnish.

Example 2

A light lubricating oil distillate and an intermediate lubricating oil distillate, derived from a Mid-Continent Louden crude, were separately phenol extracted and dewaxed as in Example 1. These were blended to a viscosity of 364 seconds Saybolt at 100° F. and treated for four hours at 15 350° F. and for one hour at 450° F. with hydrogen at 100 lbs./sd. in. pressure in the presence of 10 weight percent of 50% nickel on kieselguhr catalyst. The hydrogenated product had a color of 20 23 Robinson and a sulfur content of 0.02 weight percent. When blown with oxygen at 340° F. it absorbed approximately 9 weight percent after 1 hour to give a 99 volume percent yield of a light red colored product having a saponification number of 23, a neutralization number of 7, and a viscosity of 628 seconds Saybolt at 100° F.

The oxidized material was heated and shaken at intervals for 6 hours at 200° F. with 0.3 weight percent calcium hydroxide and 0.1 weight percent calcium oxide. By this treatment the neutralization value was reduced to 3. The product was then vacuum stripped to give a 97 volume percent yield. This partially neutralized oxidized oil was then inhibited with 1.0% of the reaction product of  $\alpha$ -pinene and  $\text{PbS}_5$ , thereby lowering the oxygen absorption rate from 2.0% in 1 hour to 0.8% in 1 hour or 1.5% in 3 hours. The oil prepared in this manner was tested in a Chevrolet engine in the manner described in Example 1, and a sample of the unoxidized oil, also with inhibitor, was likewise tested. The unoxidized oil showed a piston varnish demerit rating of 5.5-6.5, while the oxidized oil showed a demerit of 1.7. In this case also the engine operated on the oxidized oil and had a much cleaner crankcase and oil screen than when operated with the un-oxidized oil.

It is not possible at this time to give all the exact specifications for the oil to be oxidized but, in general, it is preferable to use an oil which is low in sulfur and nitrogen. These elements, along with oxygen and other materials commonly found in trace proportions, affect the oxidation rate appreciably and, therefore, affect the final product materially. The presence of small amounts of oxidation inhibitors, natural or synthetic, may effectively inhibit oxidation and/or cause sludge formation during oxidation. Thus in one experiment, proportions as low as 0.01% sulfur in the form of mercaptan or aliphatic disulfide caused sludge formation in a closed static oxidation system (Sligh oxidation at 392° F.). By extracting the same oil with a solvent (furfural or phenol) and then hydrofinishing, the same base stock was readily oxidized without sludge formation.

Hence the oil should be refined to such a degree that it can be oxidized readily to a saponification number of 20 to 70 without substantial formation of sludge or oil insoluble gums. Oils of low average molecular weight, containing about 40% of aromatic constituents, appear to give oil insoluble gums and, in general, those of lower aromatic content appear more suitable. Also, 70 75 after neutralization being heated to remove by

8  
oils capable of rapid oxidation are desirable. The drawing which accompanies this specification shows the oxidation rates for hydrofinished oils of various origins and viscosity grades, as determined by a test in which the volume of pure oxygen absorbed at 200° C. and approximately atmospheric pressure is measured, using both 10 cc. and 100 cc. oil sample tubes in the tests. Oils which absorb 800 cc. of oxygen per 10 cc. of oil in a period of not more than 100 minutes are especially desirable for the purposes of this invention.

Oils treated according to the present process may be oxidized to various degrees, but those treated to a saponification number ranging between 20 and 30 are particularly preferred for economic reasons. This product should be neutralized to as low a final neutralization number as is practicable, but various products having neutralization numbers of 4, 7, 17, 21, reduced to 1.4, 2.4, 6 and 9.4 upon treatment with basic reagent all showed reasonably good results.

Obviously, the degree and conditions of oxidation and neutralization and the agents or combinations of agents employed for neutralization may be varied within the limits previously suggested. The final products may be further modified by addition of conventional modifiers such as various antioxidants, viscosity index improvers, pour point depressants, metal deactivators, detergents, thickeners, soaps (to form greases, for example), as will be obvious to those skilled in the art.

What is claimed is:

35. 1. A lubricating oil composition prepared by contacting a solvent extracted, hydrogenated mineral lubricating oil fraction with a gas comprising free oxygen at a temperature of 200-400° F. until a product having a saponification number of at least 20 and not more than about 70 is produced, and treating the oxidized product with a neutralizing agent until the neutralization number of the same is reduced by at least 50% of its original value, said product having the property of inhibiting sludge and varnish formation in internal combustion engines operating for extended periods at low temperatures on deposit forming gasolines.
40. 2. A product according to claim 1 obtained from a lubricating oil fraction which is hydrogenated prior to oxidation in order to reduce the sulfur content to a value not greater than 0.03% by weight, to increase the color to a value of at least 18 Robinson, and to substantially increase the oxidation rate.
45. 3. A product according to claim 1 obtained by treatment of the oil with oxygen or a gas containing free oxygen at a temperature of 275-400° F.
50. 4. A product according to claim 1 in which benzoyl peroxide is used as catalyst to initiate oxidation by the gas which comprises free oxygen.
55. 5. A process which comprises treating a solvent extracted mineral base lubricating oil of low sulfur, low nitrogen, and moderately low aromatic content with a gas comprising oxygen at a temperature range between 200 and 400° F. for a period of time and under catalyst conditions such that a saponification value of at least 20 and not more than 70 is reached, then treating the oxidized oil with a neutralizing agent consisting at least in part of an alcohol capable of esterifying the oxidation product, the product 60 after neutralization being heated to remove by

distillation any portions which have boiling points lower than 350° F. at 10 mm. pressure.

6. A process according to claim 5 in which the neutralizing agent is a mixture of calcium hydroxide and calcium oxide.

7. A process according to claim 5 in which the neutralization is accomplished by first refluxing with butyl alcohol and then by treatment with a mixture of calcium hydroxide and calcium oxide.

8. A process which comprises contacting a phenol extracted hydrogenated lubricating oil fraction with oxygen at a temperature of 275-400° F. until a product having a saponification number of 20 to 70 is produced, heating the oxidized product with 10 volume percent of butyl alcohol until approximately one half of the alcohol is distilled off over a period of about 4 hours, further heating to remove the remainder of the unreacted alcohol at a temperature of 450° F. and 10 mm. pressure, heating the product for about 6 hours in the presence of 0.3 weight percent calcium hydroxide and 0.15 weight percent calcium oxide, and adding to the final product 1.0 weight percent of an oxidation inhibitor in sufficient amount to reduce the oxygen absorption rate at 350° F. of the product to less than 1% per hour.

9. Process according to claim 8 wherein the oil is oxidized to a saponification number of about 50.

10. Process according to claim 8 wherein the oil is oxidized to a saponification number of 20 to 30.

11. A product prepared by contacting a phenol extracted hydrogenated mineral lubricating oil fraction with a gas containing free oxygen at a temperature of 200-400° F. until a product having a saponification number of at least 20 and not more than 70 is produced, treating the oxidized product with a neutralizing agent until the neutralization number of the same is reduced to not more than 50% of its original value and in any case to a value not greater than 10.

12. A product according to claim 11 to which has been added an antioxidant sufficient in amount to prevent oxygen absorption when the oil is in contact with oxygen at 350° F. at a rate not greater than 1% per hour.

13. A product according to claim 11, prepared by partially neutralizing the oxygenated product with butyl alcohol and further neutralizing with a mixture of calcium hydroxide and calcium oxide.

14. A product prepared by extracting a lubricating oil distillate of about 165 seconds viscosity Saybolt at 100° F., obtained from a paraffinic type crude oil, with phenol to give an extracted oil having a viscosity index of at least 95, dewaxing the extracted oil to a pour point of about 0° F., hydrogenating the extracted, dewaxed oil until the same contains not more than 0.02% sulfur, blowing the hydrogenated oil with oxygen at about 350° F. until about 14 weight percent of oxygen has been absorbed, heating the oxidized oil with butyl alcohol until the neutralization number is reduced by at least half and in any case until it is not greater than 10, heating the partially neutralized product with a mixture of calcium hydroxide and calcium oxide until the neutralization number was reduced to not greater than 6, and adding to the oil product a sufficient amount of an antioxidant to prevent absorption of oxygen when the oil is in contact with oxygen at 350° F. at a rate greater than 1 weight percent per hour.

REGINALD K. STRATFORD.  
WILLIAM A. JONES.  
FRANK A. STUART.

References Cited in the file of this patent

UNITED STATES PATENTS

| Number    | Name      | Date          |
|-----------|-----------|---------------|
| 2,070,627 | Shoemaker | Feb. 16, 1937 |
| 2,455,337 | Jones     | Nov. 30, 1948 |
| 2,560,650 | Kronstein | July 17, 1951 |